

April 25, 1961

H. B. SNYDER ET AL

2,981,610

CHEMICAL MILLING PROCESS AND COMPOSITION

Filed May 14, 1957

2 Sheets-Sheet 1

FIG. 1



FIG. 5



FIG. 6



FIG. 2



FIG. 3



FIG. 4



FIG. 7



INVENTOR  
HERMAN BEN SNYDER  
LUDWIG M. ROSENBERG  
BY

T. W. SECRET  
ATTORNEY

April 25, 1961

H. B. SNYDER ET AL

2,981,610

CHEMICAL MILLING PROCESS AND COMPOSITION

Filed May 14, 1957

2 Sheets-Sheet 2

FIG. 8



INVENTOR  
HERMAN BEN SNYDER  
LUDWIG M. ROSENBERG  
BY

T. W. SECREST  
ATTORNEY

1

2,981,610

## CHEMICAL MILLING PROCESS AND COMPOSITION

Herman Ben Snyder and Ludwig M. Rosenberg, Seattle, Wash., assignors to Boeing Airplane Company, Seattle, Wash., a corporation of Delaware

Filed May 14, 1957, Ser. No. 659,171

9 Claims. (Cl. 41—42)

This discovery relates to the chemical milling of metal in an acid medium and, more particularly, to the chemical milling of aluminum, aluminum alloys, titanium and titanium alloys in an acid medium.

Prior to specifically discussing chemical milling we wish to point out the manner in which it distinguishes from pickling, brightening, decorative design and surface increase. Chemical milling may be considered to be controlled corrosion or controlled metal removal to form sculptured metal configurations. In chemical milling a relatively large percentage of the original metal may be rapidly removed so as to leave a minor amount of the original metal in a new configuration. As contrasted with this is pickling or scale removal whereby as much as possible of the oxide and other coating of the metal are removed but as small amount as possible of the metal is removed. In other words in pickling only the surface coating of the metal is removed. In brightening or surface polishing a minimum amount of the metal is removed to form a reflective surface, as the scale has been previously removed. Decorative designs are of a shallow depth, and approximately five mils of surface are removed by chemical action. More particularly, part of the surface is masked and the decorative design is inscribed through the masked coating. Next, a chemical solution is applied to the masked material and allowed to react to form the design. An example of this is silverware. In surface increase the object is to form a roughened surface. In order to specifically increase the surface area the same is purposely pitted by chemical action. This is done to make the surface rough enough for bonding purposes such as a metal to metal bond, for a base for paint and the manufacture of condenser plates, to name a few of the uses.

The mechanical milling of metal is well-known and extensively used throughout the metal working industries. Even though mechanical milling is extensively used it inherently has certain limitations. One of these limitations is the expensive capital investment for milling machines. Such a machine, capable of making large complicated configurations, may cost in the hundreds of thousands of dollars. In addition to the capital investment it is necessary to have skilled workmen operating these machines in order to do a creditable job on the milling of metal. Also, because of cost and man-hour requirements this type of milling is limited to certain configurations, namely, those configurations which are of a more simple or open design. However, by the skillful use of welding it is possible to build up these limited configurations into an intricate design. Because of the nature of the weld and the inherent weakness therein it is not always advisable to build up these limited basic configurations into an intricate design as the weld might rupture or the added weight may become excessive. Furthermore, with mechanical milling there usually results a relatively rough surface. Because of excessive cost the tolerance, in a recessed area, is not a close one but must be a rather large one such as in the hundredths of an inch. Also, on some of the newer metals it is impractical, because of costs due to equipment, to the time of milling involved and the technical problems involved to mechanically mill the surfaces since the metal is so tough and resistant to mechanical cutting and/or rapid

2

abrasion. For example, only casting and rough grinding can be employed with certain metals.

In recent years, as a supplement to mechanical milling, there has developed chemical milling. One of the first 5 patents to be issued for chemical milling was the patent to Sanz, United States Patent Number 2,739,047. Sanz describes the chemical milling of aluminum with a caustic solution. Basically, this patent presents the method of taking either a piece of flat stock or curved stock, masking certain predetermined areas or portions of this stock with a caustic resistant covering, and immersing the masked stock in the caustic solution. The caustic solution eats away or corrodes away the unmasked areas to form the desired configuration. Naturally, it is possible 10 to remove the stock from the caustic solution, remove the masking cover, add new masking cover and insert the stock again into the caustic solution. By such means it is possible to form intricate metallic configurations. With 15 our discovery for the use of a strong acid solution in chemical milling we find it possible to realize a more rapid action than Sanz realizes with a caustic solution; to achieve a closer tolerance than the tolerance Sanz's achieves; and, to realize a smoother surface than is possible with the caustic solution of Sanz. Also, our 20 strong acid milling solution makes it possible to work with equal ease on aluminum and its alloys be they heat treated, work hardened, cast or forged.

In United States Letters No. 2,684,291, to Wilson et al. 25 there is discussed a process for producing embossed designs on hard surface roll.

To further illustrate some of the advantages of chemical milling it is possible to achieve the same output by chemical milling with a lower capital investment than for an equal output with mechanical milling. Also, in chemical 30 milling only the application of masking material to the part to be formed requires semi-skilled labor as contrasted with the requirements of skilled labor for mechanical milling. And, more intricate configurations can be 35 formed more rapidly by chemical milling as the metal to be milled can be immersed in the reactant solution so that all parts of the metal can be acted upon simultaneously. In a specific illustration as applied to the manufacture of airplanes it is possible to reduce the weight of certain members of the airplane. As an example, 40 aluminum and alloy sheet stock may come in a thickness of 0.064 inch; however, from the design standpoint a thickness of 0.060 inch may be adequate. The original stock would not be reduced from the thickness of 0.064 inch to the thickness of 0.060 inch by mechanical milling as the cost would be too great. However, it is possible by 45 chemical milling to immerse the stock in a chemical reactant solution and reduce it to the thickness desired with ease and economy. In large airplanes this reduction in thickness may mean a considerable saving in the weight of the air frame. More particularly, for every excess 50 pound carried by the airplane there may be required from five to ten pounds of additional gross airframe weight. Therefore, if in the larger airplanes a thousand pounds of unneeded material can be saved the airframe weight can be reduced by approximately five thousand to ten 55 thousand pounds.

In another manner the configuration of a chemically milled metal can be more economically achieved than by mechanical means. For example, in the case of a waffle pattern, the necessary chemical milling can be 60 relatively easily performed as the masking material can be placed over the metal and the metal not protected by this masking material can be chemically eaten away or chemically corroded. In a like manner an object can be tapered by removing the object slowly from the chemical 65 milling solution. Also, an object having large numbers of irregularly placed recessed areas can be readily manufactured by chemical milling while the preparation of 70

a similar object by mechanical means would be time-consuming and difficult to prepare.

With this in mind it is an object of this discovery to provide a method for the chemical milling of metal, examples being intricate configurations, taper, and waffle pattern.

A further object is the provision of a method for the chemical milling of a metal and, particularly, for the chemical milling of aluminum, aluminum alloys, titanium and titanium alloys in an acid medium.

A further object is to provide a method for the chemical milling at a relatively uniform and controllable rate.

An additional object is to provide a solution for the chemical milling of metal and which solution can be controlled by standard methods of chemical analysis.

Another important object is the provision of a process for the chemical milling of metal and which process provides satisfactory surfaces having well-defined edges at better than standard machine tolerances.

A still further object is the provision of a process for chemical milling resulting in satisfactory structural and mechanical properties of the milled metal.

A still further and important object is to provide for chemical milling and which results in a satisfactorily smooth surface.

Another object is the provision of a process for chemical milling and which process produces a minimum of smut.

A further object is the provision of a process for chemical milling and which process is less expensive than mechanical milling and makes it possible to produce more intricate configurations than mechanical milling.

In the drawings:

Figure 1 is a plan view of a curved structural member illustrating two rectangular shaped recesses in the open surface thereof.

Fig. 2 is a longitudinal vertical cross-sectional view taken on line 2—2 of Fig. 1 and shows the recesses in the curved member.

Fig. 3 is a view of a mask which is placed over the non-milled structural member in Fig. 1 and protects the upper surface of said structural member, except for the two rectangular shaped openings therein, from being attacked by the chemical milling solution.

Fig. 4 is a longitudinal vertical cross-sectional view of this curved raw material from which the structural member is prepared and illustrates this raw material as being covered with protective masking coating except where the rectangular shaped recesses are to be formed.

Fig. 5, on an enlarged scale, shows the formation of a recess in metal with the aid of a masking material covering part of the metal.

Fig. 6 is an end view of a curved structural panel prior to milling; and,

Fig. 7 is an end view of the curved structural panel illustrated in Fig. 6 but after chemical milling has taken place.

Fig. 8 is a graph.

In our chemical milling solution we provide an aqueous solution having a high concentration of acid, a nitrate, a chloride, a fluoride and an acetate. In addition there may be present a citrate, a phosphate and a wetting agent. Each of these components is presumed to play a role in the chemical milling. It is to be appreciated that in solutions for milling aluminum and alloys having nitric acid in the concentration of approximately five normal, hydrochloric acid the normal, and hydrofluoric acid two normal and reaction products of these solutions with the aluminum and aluminum alloys, or solutions for milling titanium and its alloys having nitric acid in the concentration of five normal, hydrochloric acid two normal, and hydrofluoric acid five normal and reaction products of these solutions with titanium and titanium alloys the theoretical explanation of the chemical reactions may be questionable.

The milling solutions employed for milling aluminum

and its alloys and titanium and its alloys may comprise the same components. However, we believe that some of these components function differently in the milling of aluminum and its alloys than in the milling of titanium and its alloys.

Referring now to the reaction of the milling solution comprising nitric acid, hydrochloric acid and hydrofluoric acid with aluminum and its alloys, it is to be noted that all these acids separately react with aluminum. However, in the reaction of nitric acid it is noticed that if the acid is in the concentration range of about 100% that the reaction between the aluminum and the acid almost ceases. The cessation is probably due to the formation of a protective oxide of aluminum over the surface of the metal so that the acid cannot contact the unreacted metal. As contrasted with this in a moderated weak nitric acid solution there is not found this protective oxide and the acid is free to contact the metal. We believe that in our milling solution that the concentration of the nitric acid is sufficiently high so that there is formed on the surfaces of the metal an oxide layer. Turning now to the hydrochloric acid, this is of a special importance in the milling of alloys containing such alloying elements as zinc and magnesium. Also, the hydrochloric acid probably attacks the protective oxide on the surfaces of the metal to form aluminum chloride. In regard to the hydrofluoric acid there results between this component and the aluminum a terminal product, an aluminum fluoride precipitate.

The other components of the milling solution such as the citrate, the phosphate, the acetate and the wetting agent each play an important role. The acetate plays a vital role in decreasing the loss of the fluoride. For example, it is noticed that at temperatures above about 125° F. the loss of fluoride is considerable if the acetate is not present. However, if acetate be present the loss of the fluoride is lessened considerably. From this it is believed that the acetate combines or associates with the fluoride in some manner to tie up the fluoride and thereby prevent its loss by vaporization. It is realized that citric acid and a phosphate, especially disodium monohydrogen phosphate, are normally used as a buffer. However, in this strong acid solution it is believed the term buffer is not applicable as the solution is so strongly acid that very little buffering action could possibly take place. However, the citric acid and the phosphate are of considerable value and it is believed that this value arises from the fact that they function as a moderator. More specifically, the term moderator refers to the phenomenon of a partial deactivation of the surface such as the formation of a surface membrane over the metal being attacked. Such a membrane seems to act as a valve or a control on the quantity of active milling agent which can attack the surface of the metal. In regard to the wetting agent, such as an alkyl aryl sulfonate, i.e., dodecyl benzene sulfonate, this material makes it possible to achieve a better surface. The wetting agent probably functions, by reducing the surface tension, to allow the gases produced by the action of the solution on the metal to more readily escape from the surface and therefore to permit a more uniform concentration of milling solution to react with the surface of the metal. It is realized that if the gases do not readily escape then that portion of the metal covered by the gases will not be reacted upon in the same manner as that portion not covered by the gas bubbles and therefore there would result an uneven or a less smooth surface.

In the milling of aluminum and its alloys with these milling solutions we have found that once the milling solution is raised to a temperature above about 100° F. and reacted with the metal that the temperature of the solution should not be allowed to decrease below approximately 100° F. If the temperature is allowed to decrease to a value below approximately 100° F. and then increased above this indicated temperature the re-

action of the solution with the metal is a different one than if the solution had not been allowed to cool and then been reheated. We therefore believe that it is advisable that if the solution upon being raised to a temperature above 100° F. and reacted with metal then that solution should thereafter be maintained at a temperature above 100° F.

In the milling of aluminum and its alloys with these solutions we consider that hydrogen pickup or hydrogen embrittlement is not a problem. Actually, the hydrogen released cannot effectively pass through the protective oxide layer on the surface of the metal to penetrate into the same and to cause embrittlement.

Turning now to the reaction of the milling solution comprising nitric acid, hydrochloric acid and hydrofluoric acid with titanium and its alloys it is to be noted that of these three only hydrofluoric acid reacts with titanium. The other two acids, hydrochloric and nitric, are not capable of attacking titanium to as to be the basis of an economical milling solution. However, it is to be realized that these two acids play an important role in the milling of titanium and its alloys. Turning first to the action of the nitric acid it is noted that a solution having a high concentration of hydrofluoric acid rapidly corrodes titanium. In fact, the corrosion rate is often so rapid that a controlled product cannot be realized. However, with the addition of nitric acid a controlled product can be made. We believe that in this regard that the nitric acid reacts with the titanium to form a protective oxide or oxides on the surface of the metal. The protective oxide functions to limit the passage of hydrofluoric acid to the metal. By so limiting the reaction of hydrofluoric acid with the metal there is regulated the corrosion of the titanium. As a result there is a regulated milling rate. In addition to regulating the milling rate the nitric acid acts to cut down or eliminate hydrogen contamination. Hydrogen contamination may adversely affect structural properties of titanium and its alloys. Returning now to the oxides of titanium these react with hydrofluoric acid to form complexes of titanium, oxygen, and fluorine. These complexes or compounds are soluble in water. The value of the soluble products resides in forming better and more uniform milled product as a solution free of a precipitate is of a more uniform concentration. Or, in other words, in a solution having a precipitate there are concentration gradients making it more difficult to achieve a uniform product. Turning now to the hydrochloric acid, this component attacks some of the alloying elements, viz., aluminum, manganese, vanadium, etc., and thereby plays a vital role.

In these solutions for the milling of titanium and its alloys the actions of the acetate, the citrate, the phosphate and the wetting agent are believed to be the same as in the reaction with aluminum and its alloys and therefore will not be described again.

We have noticed in the milling of titanium and its alloys, as contrasted with the milling of aluminum and its solutions, that the temperatures of the milling solution can be raised to above 100° F. and the solution reacted, the temperatures lowered to room temperature and again raised without affecting the reaction properties of the solution. Also, in the milling of titanium and its alloys by these solutions a smoothness value of about 15 R.M.S. or better can be realized. Of course, sufficient reaction time must be given to smooth out the original rough surfaces. R.M.S. means "root mean square" and is expressed in micro inches of amplitude of surface variations. Finally, as a sidelight on the reaction of these solutions it was noted that with the alloy, 6Al-4V-Ti, that there was not formed a precipitate of aluminum. This indicates that the reaction with titanium and its alloys is different than with aluminum and its alloys.

In the milling solutions we prepared, the nitrate was added as hydrogen nitrate or nitric acid, the fluoride as hydrogen fluoride or hydrofluoric acid, the acetate as

hydrogen acetate or acetic acid, the chloride as hydrogen chloride or hydrochloric acid, the citrate as hydrogen citrate or citric acid and the phosphate as disodium monohydrogen phosphate.

In the milling process there are a number of factors determining the milling rate. Some of these factors are temperature, concentration of components, heat transfer, evaporation, agitation, volume of milling solution to surface area of metal, and so forth. Briefly, it is readily realized that the role of the temperature is very important. Generally speaking a ten degree rise in temperature, on the Kelvin scale, indicates a doubling in the reaction rate. Therefore, it is possible to achieve with a relatively dilute or weak milling solution a milling rate at a higher temperature equal to the milling rate of a more concentrated solution at lower temperature. Also, it is apparent that the concentration of the reactant plays a very vital and important role in chemical milling. This is of importance in the fact that a control of the milling can be obtained by control of the temperature. Heat transfer is of utmost importance as good heat transfer precludes the possibility of a local build-up of temperatures and also is essential for proper control of the milling rate. The local build-up of temperature means that in that particular area the reaction rate will be higher and more metal will be removed or corroded away. This uneven removal of the metal can result in uneven surfaces, pitting and tapering. Evaporation is of importance in that the evaporation of a vital component, viz., such as a fluoride, means that the reaction rate will change and the life of the milling solution and the uniformity of the reaction rate cannot be as closely controlled as if evaporation had not taken place. Of great importance in the chemical milling of metal is the agitation of the solution. A well-agitated solution gives more even and uniform results than one which is not agitated. This agitation may be in the form of mechanical agitation whereby the metal undergoing the milling action is vibrated or shaken back and forth in the milling bath. Another form of agitation may be that of the milling solution itself whereby it is agitated by a gas bubbling through it. And, a still further and desirable form is that of ultrasonic vibration whereby high-frequency ultrasonic agitation is applied to the solution or to the metal undergoing reaction so as to break up any localized variations in solution concentration. This also serves to avoid gas accumulation on the metal surface. Furthermore, the volume of the reacting chemical milling solution in proportion to the surface area of the material undergoing reaction can be of considerable importance. If the volume to surface ratio is rather low it is possible that the reactive components available at the milling surface will be rapidly exhausted and therefore there will be an uneven reaction rate and possibly an uneven removal of the metal affecting the quality of the finished product. Therefore, a large ratio of volume to surface area would probably give a more constant reaction rate and thus permit closer tolerances on the finished product.

To more particularly illustrate our discovery and especially the effects of the variation of the concentration of components and also the effect of the variation of the temperature we herewith present specific detailed examples. These examples are to be taken for illustrative purposes only and are not to be taken as limitations on the invention. In these examples the specifically enumerated components were utilized. More particularly, concentrated nitric acid of a specific gravity of approximately 1.42 and of a concentration of 68-70%; hydrochloric acid of a specific gravity of approximately 1.19 and a concentration of 38%; glacial acetic acid of a specific gravity of 1.055. Also, there were prepared a citric acid solution and a disodium monohydrogen phosphate solution. These two solutions were prepared by heating water to its boiling point and adding an excess of citric acid to one

and the disodium monohydrogen phosphate to the other. The solutions were allowed to cool to room temperature and the supernatant liquid decanted from the precipitate. Saturated solutions of oxalic and boric acids were prepared in a similar manner.

Turning now to specific examples of the invention proper a fundamental milling solution was prepared and to this solution there were added various components to make different milling solutions for testing purposes. The

cates that the hydrofluoric acid was an active agent in the milling. To solutions such as D there was added citric acid and disodium monohydrogen phosphate to prepare solutions E and F. A comparison of D, E, and F, in an increasing temperature range, 112-139° F., 116-152° F., and 142-206° F., respectively, shows an increase in the milling rates with an increase in temperature. Specifically, D milled at the rate of about 0.9 mil per minute, E at 2.0 and F at 3.0.

Table I

| Variable                                       | A           |       | B           |       | C           |       | D           |       | E           |       | F           |       |
|------------------------------------------------|-------------|-------|-------------|-------|-------------|-------|-------------|-------|-------------|-------|-------------|-------|
|                                                | Wt. Percent | N     | Wt. Percent | N     | Wt. Percent | N     | Wt. Percent | N     | Wt. Percent | N     | Wt. Percent | N     |
| HNO <sub>3</sub> (68-70%)                      | 20.2        | 2.4   | 20.1        | 2.4   | 20.1        | 2.4   | 20.0        | 2.3   | 19.9        | 2.3   | 19.9        | 2.3   |
| HCl (38%)                                      | 7.5         | 0.8   | 7.5         | 0.8   | 7.5         | 0.8   | 7.4         | 0.7   | 7.4         | 0.7   | 7.4         | 0.7   |
| Acetic acid (glacial)                          | 2.3         | 0.4   | 2.3         | 0.4   | 2.3         | 0.4   | 2.3         | 0.4   | 2.3         | 0.4   | 2.3         | 0.4   |
| HF (60%)                                       | 5.1         | 1.7   | 5.1         | 1.7   | 5.1         | 1.7   | 6.4         | 1.9   | 6.4         | 1.9   | 6.4         | 1.9   |
| H <sub>2</sub> O                               | 64.9        | ----- | 64.5        | ----- | 64.5        | ----- | 64.4        | ----- | 64.4        | ----- | 64.4        | ----- |
| Citric acid (sat'd sol'n)                      | -----       | 0.4   | -----       | 0.4   | -----       | 0.4   | -----       | 0.4   | -----       | 0.4   | -----       | 0.4   |
| Na <sub>2</sub> HPO <sub>4</sub> (sat'd sol'n) | -----       | 0.2   | -----       | 0.2   | -----       | ----- | -----       | 0.1   | -----       | 0.1   | -----       | 0.1   |
| Metal <sup>1</sup>                             | -----       | ----- | -----       | ----- | -----       | ----- | -----       | ----- | -----       | ----- | -----       | ----- |
| Temperature ° F                                | 123-132     | ----- | 123-135     | ----- | 160-195     | ----- | 112-139     | ----- | 116-152     | ----- | 142-206     | ----- |
| R.M.S.                                         | 20-26       | ----- | 20-26       | ----- | 30-40       | ----- | 20-25       | ----- | 22-30       | ----- | 30-50       | ----- |
| Milling rate (mils/min.)                       | 0.7         | ----- | 0.8         | ----- | 2.0         | ----- | 0.9+        | ----- | 2.0         | ----- | 3.0         | ----- |

<sup>1</sup> A heat treated aluminum alloy such as 7075S-T6, weight of 0.045 g./in.<sup>2</sup> mil.

results of these tests are presented in following Table I. In this table there are listed the components of the milling solution, the temperature of milling, the smoothness of the milled object expressed in R.M.S. terms and the milling rate. For each individual test there is presented the percentage by weight of each component and the normality of the stronger acids.

Referring to Table I it is seen that solution A comprised nitric acid, hydrochloric acid, acetic acid, hydrofluoric acid and water. This solution was used to mill an aluminum alloy such as 7075S-T6, weight of 0.045 gram per (square inch mil) volume, in the temperature range of 123-132° F. The milling rate was about 0.7 mil per minute and the smoothness was in the range of 20 to 26. To solutions such as A there were added both saturated citric acid solution and saturated disodium monohydrogen phosphate solution to make solutions B and C. The aluminum alloy was milled by B at a temperature in the range of 123-134° F. The comparison of B and A shows that B milled the alloy at a rate of about 0.8 to approximately 0.7 mil per minute for A. The smoothness of the alloys on metal milled by B and A were the same, being in the range of 20 to 26 R.M.S. A comparison of C and B, C being at a temperature in the range of 160-195° F. and B in the range of 123-134° F., shows that C milled faster than B, about 2.0 compared to 0.8 mil per minute. This is to be expected due to the higher milling temperature of C in comparison with B. A solution such as A was varied by the addition thereto of hydrofluoric acid to raise the concentration thereof to about 1.9 normal so as to make solution D. A comparison of D and A shows that D milled in the same temperature range, at a faster rate of about 0.9 instead of 0.7 mil per minute. This indi-

30 water in predetermined quantities so as in effect to dilute the concentration of the active components. Also, to solutions similar to the most dilute solution there was added additional hydrofluoric acid. The metal tested by this solution was an alloy of aluminum having a density of about 0.045 gram per (square inch mil) volume. The most fundamental solution comprised nitric acid in the strength of approximately 2.9 normal, hydrochloric acid at approximately 1.0 normal and hydrofluoric acid at about 2.2 normal. This solution is referred to as A. To similar solutions there were added various quantities of 35 water to make solutions B, C, D, E, and F. The active components in each of these solutions remained the same in quantity although, as realized, less in concentration. For example in solution A the concentration of nitric acid was 2.9 normal and in solution F was 1.3 normal. For hydrochloric acid in solution A the normality was 1.0 and in solution F 0.44 normal, and for hydrofluoric acid in A the normality was 2.2 and in F it was 0.9. These 40 were the limits on the concentration of the most acidic components. The temperature range in which the chemical milling was conducted, except for solution A, was substantially the same for all the solutions. More particularly, in solution A the temperature of the solution ranged from 145-210° F. However, in solutions B through F the temperature ranged from approximately 140° F. to about 162° F. The results of this series of 45 chemical milling solutions is presented in the following Table II.

Table II

| Variable                  | A           |       | B           |       | C           |       | D           |       | E           |       | F           |       | G           |       | H           |       |
|---------------------------|-------------|-------|-------------|-------|-------------|-------|-------------|-------|-------------|-------|-------------|-------|-------------|-------|-------------|-------|
|                           | Wt. Percent | N     | Wt. Percent | N     | Wt. Percent | N     | Wt. Percent | N     | Wt. Percent | N     | Wt. Percent | N     | Wt. Percent | N     | Wt. Percent | N     |
| HNO <sub>3</sub> (68-70%) | 24.6        | 2.9   | 20.2        | 2.4   | 17.2        | 2.0   | 14.9        | 1.7   | 13.2        | 1.5   | 11.8        | 1.3   | 11.7        | 1.3   | 11.7        | 1.3   |
| HCl (38%)                 | 9.1         | 1.0   | 7.5         | 0.8   | 6.4         | 0.7   | 5.5         | 0.6   | 4.9         | 0.5   | 4.4         | 0.44  | 4.3         | 0.44  | 4.3         | 0.44  |
| Acetic acid (glacial)     | 2.8         | 0.5   | 2.3         | 0.4   | 2.0         | 0.3   | 1.7         | 0.28  | 1.6         | 0.24  | 1.3         | 0.22  | 1.3         | 0.22  | 1.3         | 0.22  |
| HF (60%)                  | 6.5         | 2.2   | 5.3         | 1.7   | 4.5         | 1.5   | 3.9         | 1.2   | 3.5         | 1.1   | 3.1         | 0.9   | 4.3         | 1.4   | 4.3         | 1.4   |
| H <sub>2</sub> O          | 57.0        | ----- | 61.7        | ----- | 69.9        | ----- | 73.9        | ----- | 76.8        | ----- | 79.3        | ----- | 79.8        | ----- | 79.8        | ----- |
| Metal <sup>1</sup>        | -----       | ----- | -----       | ----- | -----       | ----- | -----       | ----- | -----       | ----- | -----       | ----- | -----       | ----- | -----       | ----- |
| Temperature ° F           | 145-210     | ----- | 162         | ----- | 151         | ----- | 149-145     | ----- | 144-142     | ----- | 143-140     | ----- | 135-134     | ----- | 121-120     | ----- |
| R.M.S.                    | 25-40       | ----- | 25-35       | ----- | 20-30       | ----- | 20-30       | ----- | 20-25       | ----- | 18-35       | ----- | 19-26       | ----- | 18-25       | ----- |
| Milling rate mils/min.    | 4.7         | ----- | 1.3         | ----- | 0.8+        | ----- | 0.8         | ----- | 0.6+        | ----- | 0.5         | ----- | 0.5         | ----- | 0.4         | ----- |

<sup>1</sup> A heat treated alloy of aluminum such as 7075S-T6, weight of about 0.045 g./in.<sup>2</sup> mil.

Referring to Table II it is seen that the chemical milling rate for these solutions decreased with the addition of water. As expected solution A milled at the fastest rate of approximately 4.7 mils per minute, B at the rate of approximately 1.3, C at about 0.8 plus, D at about 0.8 minus, E at about 0.6, and F at about 0.5 mil per minute. This illustrates that the addition of water to the fundamental solution decreased the concentration of the active components and with this decrease in the concentration of the active components for a given temperature range the milling rate decreased. To solutions such as F there was added additional hydrofluoric acid to make solutions G and H. More particularly, the concentration of the hydrofluoric acid in solution F was about 0.9 normal and in solutions G and H it was about 1.4 normal. The temperature ranges for which the milling was done with solutions F, G and H was such that F was in the range of 140-143° F., G at about 135° F., and H at about 121° F. The milling rate for these three solutions was substantially the same as F and G milled at the rate of about 0.5 mil per minute while H milled at the rate of about 0.4 mil per minute. It is seen that with the higher concentration of hydrofluoric acid in G as compared to F but at a lower milling temperature of G to F that the milling rates of these two solutions were substantially the same. These solutions indicate that it is possible to mill at the same rate at a lower temperature if there is a higher concentration of hydrofluoric acid present. In regard to a comparison of G and H it is seen that a decrease in the temperature for the same milling solution results in a decrease in the milling rate.

Another series of chemical solutions was prepared comprising nitric acid, hydrochloric acid, acetic acid, hydrofluoric acid, citric acid, disodium monohydrogen phosphate, and water. Again, a fundamental solution was prepared and this solution was varied in a number of ways to determine the effect of the addition of hydrofluoric acid, the effect of temperature upon the chemical milling solution and the effect of the dilution of the concentration of the active components. The metal used in the chemical milling action was a heat treated alloy of aluminum having a density of about 0.045 gram per (square inch mil) volume. The results of this series of tests are illustrated in tabular form in following Table III.

Table III

| Variable                         | A           |       | B           |       | C           |       | D           |       | E           |       | F           |       | G           |       |
|----------------------------------|-------------|-------|-------------|-------|-------------|-------|-------------|-------|-------------|-------|-------------|-------|-------------|-------|
|                                  | Wt. Percent | N     | Wt. Percent | N     | Wt. Percent | N     | Wt. Percent | N     | Wt. Percent | N     | Wt. Percent | N     | Wt. Percent | N     |
| HNO <sub>3</sub> (68-70%)        | 13.3        | 1.5   | 13.0        | 1.5   | 13.0        | 1.5   | 8.0         | 1.0   | 8.9         | 1.0   | 8.9         | 1.0   | 8.7         | 1.0   |
| HCl (38%)                        | 10.0        | 1.0   | 9.7         | 1.0   | 9.7         | 1.0   | 6.7         | 0.67  | 6.7         | 0.67  | 6.7         | 1.0   | 6.5         | 1.0   |
| Acetic acid (glacial)            | 3.0         | 0.5   | 2.9         | 0.5   | 2.9         | 0.5   | 1.9         | 0.33  | 1.9         | 0.33  | 1.9         | 0.32  | 1.9         | 0.32  |
| HF (60%)                         | 1.3         | 0.4   | 3.8         | 1.2   | 3.8         | 1.2   | 2.6         | 0.8   | 2.6         | 0.8   | 2.6         | 0.8   | 5.2         | 1.9   |
| Citric acid (sat'd sol'n)        | 1.1         | —     | 1.1         | —     | 1.1         | —     | 0.8         | —     | 0.8         | —     | 0.8         | —     | 0.7         | —     |
| NaHPO <sub>4</sub> (sat'd sol'n) | 0.4         | —     | 0.4         | —     | 0.4         | —     | 0.3         | —     | 0.3         | —     | 0.3         | —     | 0.2         | —     |
| H <sub>2</sub> O                 | 71.0        | —     | 69.1        | —     | 69.1        | —     | 78.8        | —     | 78.8        | —     | 78.8        | —     | 76.8        | —     |
| Metal <sup>1</sup>               | —           | —     | —           | —     | —           | —     | —           | —     | —           | —     | —           | —     | —           | —     |
| Temperature ° F.                 | Room        | 90    | 150         | 120   | 150         | 150   | 150         | 150   | 150         | 150   | 150         | 150   | 135         | 135   |
| R.M.S.                           | 37-42       | 43-55 | 32-42       | 25-33 | 25-33       | 28-35 | 28-35       | 25-35 | 25-35       | 25-35 | 25-35       | 25-35 | 30-40       | 30-40 |
| Milling rate (mils/min.)         | 0.2—        | 0.3—  | 0.7+        | 0.3—  | 0.3+        | 0.3+  | 0.3+        | 0.3+  | 0.3+        | 0.3+  | 0.3+        | 0.3+  | 0.8+        | 0.8+  |

<sup>1</sup> An alloy of aluminum having a weight of about 0.045 g./in.<sup>2</sup> mil.

Referring to the above Table III it is seen that the fundamental solution A comprised nitric acid at about 1.5 normal, hydrochloric acid at about 1.0 normal and hydrofluoric acid at about 0.4 normal. The metal was chemically milled at room temperature and the solution showed a milling rate of approximately 0.2 mil per minute. To solutions such as A there was added hydrofluoric acid to prepare solutions B and C having a concentration of hydrofluoric acid of about 1.2 normal. Solution B was used for milling at a temperature of about 90° F. and solution

to make solution G by the addition to F of hydrofluoric acid. This raised the concentration of the hydrofluoric acid from approximately 0.8 normal in F to approximately 1.9 normal in G. The milling temperature of G was approximately fifteen degrees (15° F.) less than the milling temperature of solution F, viz., 135° F. as compared with 150° F. However, the addition of the hydrofluoric acid raised the milling rate appreciably as is seen from the fact that the milling rate for solution G was approximately 0.8 mil per minute as compared with about 0.4 mil per minute.

for solution F. This considerable increase in the milling rate of solution G indicates that the addition of hydrofluoric acid is of prime importance to the milling solution and that within reasonable limits the higher the concentration of the hydrofluoric acid present the greater the milling rate.

As a side light on solution G it was decided that other alloys and metals should be subjected to the milling action of this solution. Therefore, aluminum and alloys such as 2014, 2017, 5052, 6061, 7075, 7178, 2024 and 1100; carbon steels such as 1025, 1090; alloy steels such as 4130, 4340 and 4130 modified; stainless steel such as 302; and, heat treatable stainless steel such as 17-7PH, 17-4PH, and AM350 were chemically milled. A more particular and complete definition of these metals can be found in the "Metals Handbook" published by the American Society for Metals, Cleveland, Ohio. In a qualitative manner the milling solution G rapidly removed the metal and produced a satisfactory smooth surface. The milling action of the solution was determined in a qualitative manner whereby the alloy was submerged in the solution for a certain period of time and the action of the solution on the alloy was determined by visual inspection.

Another series of test solutions was prepared comprising the components nitric acid, hydrochloric, acetic acid, hydrofluoric acid, citric acid, disodium monohydrogen phosphate and water. The metal which was milled by various solutions of this fundamental composition of matter was a heat treated alloy of aluminum having a density of 0.045 gram per (square inch mil) volume, g./in.<sup>2</sup> mil. There were prepared seven different test solutions for this particular series and the results of these tests are tabulated in Table IV, which follows.

Table IV

| Variable                                       | A           |       | B           |       | C           |       | D           |       | E           |      |
|------------------------------------------------|-------------|-------|-------------|-------|-------------|-------|-------------|-------|-------------|------|
|                                                | Wt. Percent | N     | Wt. Percent | N     | Wt. Percent | N     | Wt. Percent | N     | Wt. Percent | N    |
| HNO <sub>3</sub> (68-70%)                      | 25.6        | 3.2   | 25.0        | 3.1   | 25.0        | 3.1   | 25.0        | 3.1   | 17.4        | 1.3  |
| HCl (38%)                                      | 9.5         | 1.1   | 9.3         | 1.1   | 9.3         | 1.1   | 9.3         | 1.1   | 6.4         | 0.6  |
| Acetic acid (glacial)                          | 2.9         | 0.53  | 2.8         | 0.52  | 2.8         | 0.52  | 2.8         | 0.52  | 2.0         | 0.35 |
| HF (60%)                                       | 1.3         | 0.4   | 3.8         | 1.3   | 3.8         | 1.3   | 3.8         | 1.3   | 2.6         | 0.87 |
| Citric acid (sat'd sol'n)                      | 1.1         | —     | 1.0         | —     | 1.0         | —     | 1.0         | —     | 0.7         | —    |
| Na <sub>2</sub> HPO <sub>4</sub> (sat'd sol'n) | 0.4         | —     | 0.3         | —     | 0.3         | —     | 0.3         | —     | 0.2         | —    |
| H <sub>2</sub> O                               | 59.2        | —     | 57.8        | —     | 57.8        | —     | 57.8        | —     | 70.8        | —    |
| Metal <sup>1</sup>                             |             |       |             |       |             |       |             |       |             |      |
| Temperature ° F.                               | Room        | 90    |             | 115   |             | 150   |             | 120   |             |      |
| R.M.S.                                         | 38-45       | 30-45 |             | 30-35 |             | 28-35 |             | 30-40 |             |      |
| Milling rate (mils/min.)                       | 0.2—        | 0.3+  |             | 0.7+  |             | 1.1   |             | 0.3—  |             |      |

<sup>1</sup> A heat treated alloy of aluminum such as 7075S-T6, having a weight of about 0.045 g./in.<sup>2</sup> mil.

The fundamental solution in this series was A which comprised a high percentage of nitric acid, being approximately 3.2 normal. The percentage of hydrofluoric acid was low being in the range of about 0.4 normal. The metal was chemically milled by solution A at approximately room temperature and at a milling rate of nearly 0.2 mil per minute. From solutions such as A three other solutions were prepared by increasing the concentration

of the hydrofluoric acid from approximately 0.4 normal to approximately 1.3 normal. These three other solutions were B, C and D. As solutions, B, C and D did not differ fundamentally from each other but as chemical milling solutions they differed from each other in respect to the milling temperature. More particularly, B was held at the temperature of about 90° F., C at a temperature of approximately 115° F., and D at a temperature of about 150° F. From Table IV it is seen that the milling rate of B was less than either C or D. This was to be expected as the milling temperature was lower. Also, C was less than D for the same reason. A comparison of solutions B and A, it being assumed that the temperature of A was substantially room temperature, indicates that the addition of the hydrofluoric acid increased the milling rate of B over A. This was to be expected. To a solution such as C there was added water to make a more dilute solution E in terms of the active components. For example, the concentration of the hydrofluoric acid was decreased from approximately 1.3 normal to approximately 0.9 normal. These two solutions, C and E, were used for milling at substantially the same temperatures, being in the range of 115 to 120° F. The addition of the water substantially decreased the milling rate of E in comparison with C as the milling rate of E was approximately 0.3 mil per minute while the milling rate of C was approximately 0.7 mil per minute.

Another solution was prepared comprising nitric acid, hydrochloric acid, acetic acid, hydrofluoric acid, citric acid, disodium monohydrogen phosphate, and water. In the initial solution A the concentration of the nitric acid was relatively high being approximately 4.8 normal and

Table V

| Variable                                       | A           |       | B           |       | C           |       | D           |       | E           |       | F           |       | G           |       | H           |       |
|------------------------------------------------|-------------|-------|-------------|-------|-------------|-------|-------------|-------|-------------|-------|-------------|-------|-------------|-------|-------------|-------|
|                                                | Wt. Percent | N     | Wt. Percent | N     | Wt. Percent | N     | Wt. Percent | N     | Wt. Percent | N     | Wt. Percent | N     | Wt. Percent | N     | Wt. Percent | N     |
| HNO <sub>3</sub> (68-70%)                      | 37.2        | 4.74  | 36.3        | 4.64  | 36.3        | 4.64  | 36.3        | 4.64  | 25.4        | 3.12  | 25.4        | 3.12  | 24.6        | 3.00  | 24.0        | 2.96  |
| HCl (38%)                                      | 0.1         | 1.09  | 8.9         | 1.06  | 8.9         | 1.06  | 8.9         | 1.06  | 6.3         | 0.71  | 6.3         | 0.71  | 9.6         | 1.13  | 9.5         | 1.12  |
| Acetic acid (glacial)                          | 2.8         | 0.53  | 2.7         | 0.52  | 2.7         | 0.52  | 2.7         | 0.52  | 1.9         | 0.35  | 1.9         | 0.35  | 1.8         | 0.35  | 1.8         | 0.34  |
| HF (60%)                                       | 1.2         | 0.42  | 3.6         | 2.09  | 3.6         | 2.09  | 3.6         | 2.09  | 2.5         | 1.41  | 2.5         | 1.41  | 2.5         | 1.40  | 4.0         | 2.2   |
| Citric (sat'd sol'n)                           | 1.0         | —     | 1.0         | —     | 1.0         | —     | 1.0         | —     | 0.7         | —     | 0.7         | —     | 0.7         | —     | 0.7         | —     |
| Na <sub>2</sub> HPO <sub>4</sub> (sat'd sol'n) | 0.3         | —     | 0.3         | —     | 0.3         | —     | 0.3         | —     | 0.2         | —     | 0.2         | —     | 0.2         | —     | 0.2         | —     |
| H <sub>2</sub> O                               | 48.3        | —     | 47.0        | —     | 47.0        | —     | 47.0        | —     | 62.9        | —     | 62.9        | —     | 60.6        | —     | 59.5        | —     |
| Metal <sup>1</sup>                             |             |       |             |       |             |       |             |       |             |       |             |       |             |       |             |       |
| Temperature ° F.                               | 35-42       | 30-40 | 90          | 115   | 150         | 120   | 150         | 120   | 150         | 120   | 150         | 120   | 140         | 140   | 135         | 135   |
| R.M.S.                                         | 30-40       | 30-40 | 30-35       | 35-45 | 35-45       | 32-42 | 30-40       | 30-40 | 30-45       | 30-45 | 30-40       | 30-40 | 30-40       | 30-40 | 30-40       | 30-40 |
| Milling rate (mils/min.)                       | 0.2         | 0.4   | 0.7+        | 0.7+  | 1.4         | 0.2+  | 0.4         | 0.2+  | 0.4         | 0.2+  | 0.4         | 0.2+  | 0.2+        | 0.2+  | 0.9+        | 0.9+  |

<sup>1</sup> A heat treated aluminum alloy such as 7075S-T6 and having a weight of about 0.045 g./in.<sup>2</sup> mil.

As is seen from Table V in solution A the concentration of the hydrofluoric acid was approximately 0.4 normal. The milling of the metal at room temperature was as the rate of approximately 0.2 mil per minute. To a solution such as A there was added hydrofluoric acid so as to raise the concentration of this component from approximately 0.4 normal to about 2.1 normal. Three solutions were prepared in this manner, these being B, C and D. These solutions were employed for milling the indicated metal and each was employed at a different temperature. For example, B was at approximately 90° F., C at about 115° F., and D at about 150° F. In each instance the solution at the higher temperature milled the metal at a faster rate. For example, B milled the metal at approximately 0.4 mil per minute, C at about 0.7 and D at about 1.4 mils per minute. Also, the smoothness value or root mean square of the metal was substantially the same for these three, being in the range of approximately 30 to 45 millionths of an inch in amplitude. To solutions such as the solutions B, C or D, there was added water so as to lower the concentration of the more active components such as nitric acid, hydrochloric acid, and hydrofluoric acid. Two solutions were prepared in this manner. These were E and F. The solution E was employed for milling at approximately 120° F. and solution F at about 150° F. For our purposes the solutions C and E can be compared as they differed mainly by E being less concentrated than C. However, the milling temperatures of these two solutions were substantially the same, about 115° to 120° F. It is seen by this comparison that E milled at a lower rate than C, approximately 0.2 mil per minute to approximately 0.7 mil per minute. This means that the addition of the water substantially lowered the milling rate. As further evidence in this regard a comparison of solutions F and D indicates the same, as these two solutions were substantially the same except that F contained more water than D and therefore the concentration of the active components was less. Again, the milling rate of the more dilute or less concentrated solution is less than the milling rate of the concentrated solution. For example, the solution F milled at approximately 0.4 mil per minute while the solution D at about 1.4 mils per minute. The effectiveness of the concentration of the hydrochloric acid was brought out in the comparison of solutions G and E whereby solution G was substantially the same as solution E except that G contained more hydrochloric acid. Also, G, 0.2 mil per minute, was employed as a milling solution at approximately 140° F. as compared to E, also 0.2 mil per minute, at about 120° F. It is seen that the milling rate of these two solutions was substantially the same, approximately 0.2 mil per minute. This indicates that in the concentrations of the components employed in E and F that the hydrochloric acid played a secondary role. The concentration of the hydrofluoric acid was further investigated by comparing solutions G and H wherein the hydrofluoric acid concentration of H was raised over that of G from about 1.4 normal to about 2.2 normal. The temperatures of these two solutions were approximately the same, being in the range of about 140° to 135° F. However, it is noted that solution H milled at a rate of about 0.9 mil per minute while the solution G milled at a rate of approximately 0.2 mil per minute. At the concentration of the components in the solutions G and H it is seen that the higher the concentration of the hydrofluoric acid present the greater the chemical milling rate.

Another series of chemical milling solutions for the milling of aluminum was prepared. This series of solutions comprised nitric acid, hydrochloric acid, acetic acid,

hydrofluoric acid, disodium monohydrogen phosphate, oxalic acid, a wetting agent such as sodium salt of decyl benzene sulfonic acid and water. A summary of these milling solutions and their reaction with aluminum is presented in following Table VI. Prior to discussing the solutions it will be stated that the oxalic acid was a saturated aqueous solution prepared by heating water to the boiling point, adding an excess of oxalic acid, cooling, and decanting the clear supernatant liquid. In this table it is seen that solutions A and B were substantially the same, the only difference being that A was used for milling at 70° F. and B at 140° F. More particularly, in A and B the nitric acid was approximately 0.1 normal, the hydrochloric acid about 0.1 normal, and the hydrofluoric acid a little over three normal. The milling rate for solution A was about 0.3 mil per minute and for solution B about 2.0 mils per minute. The metal milled was heat treated aluminum alloy such as 7075-T6 and having a weight of about 0.045 gram per (square inch mil) volume, 0.045 g./in.<sup>2</sup> mil. Solution A produced a surface roughness in the range of 35-40 R.M.S., and solution B a roughness in the range of 47-53 R.M.S. Turning now to solutions C and D, which were the same in composition but were used for milling at two different temperatures, it is seen that these solutions comprised about 0.1 normal nitric acid, hydrochloric acid being about 2.2 normal and hydrofluoric acid being about 3.2 normal. Solution C was used for milling at 70° F. and had a milling rate of 0.8 mil per minute while solution D was used for milling at 120° F. and had a much higher milling rate of 4 mils per minute. Solution C gave a better surface than D, having a roughness value in the range of 36-40 R.M.S. and D a value in the range of 50-55 R.M.S. A comparison of C with A shows that for an increase in the concentration of the hydrochloric acid with the concentration of the other components remaining substantially the same that the milling rate increased. In fact, for the same temperatures the milling rate of C was over twice as great as the milling rate of A, and even for a decrease in temperature of D with respect to B the milling rate of D was approximately twice the milling rate of B. This indicates that there should be a minimum concentration of hydrochloric acid present to cut the alloying elements. Below this minimum concentration the milling rate is depressed. Another set of solutions was prepared, E and F, wherein the concentration of the nitric acid was raised to 3.1 normal, the concentration of hydrochloric was 0.1 normal, and hydrofluoric was decreased to 1.6 normal. Composition E was used for milling at 100° F. and milled at the rate of 0.1 mil per minute and solution F was used for milling at 160° F. and milled at the rate of 1.3 mils per minute. The R.M.S. value of E was in the range of 28-33 while for F was in the range of 41-47. A comparison of E with A, B, C and D indicates that with an increase in the nitric acid concentration that the milling rate was decreased somewhat. However, there was a decrease in the concentration of the hydrochloric and hydrofluoric acid which may also be interpreted to mean that the milling rate decreases with the decrease in the concentrations of these components. A comparison of E and F shows that with a sufficiently high milling temperature the effect of a low concentration of components can be overcome so as to achieve a satisfactory milling rate.

Another series of milling solutions was formulated and in this series the concentration of the hydrofluoric acid was varied from zero to approximately 2.7 normal. For this series of milling solutions see following Table VII.

Table VI

| Variable                                       | A           |     | B           |     | C           |     | D           |     | E           |     | F           |     |
|------------------------------------------------|-------------|-----|-------------|-----|-------------|-----|-------------|-----|-------------|-----|-------------|-----|
|                                                | Wt. Percent | N   | Wt. Percent | N   | Wt. Percent | N   | Wt. Percent | N   | Wt. Percent | N   | Wt. Percent | N   |
| HNO <sub>3</sub> (68-70%)                      | 1           | 0.1 | 1           | 0.1 | 1           | 0.1 | 1           | 0.1 | 25          | 3.1 | 25          | 3.1 |
| HCl (38%)                                      | 1           | 0.1 | 1           | 0.1 | 20          | 2.2 | 20          | 2.2 | 1           | 0.1 | 1           | 0.1 |
| Acetic acid (glacial)                          | 10          | 1.7 | 10          | 1.7 | 2           | 0.4 | 2           | 0.4 | 5           | 0.9 | 5           | 0.9 |
| HF (60%)                                       | 10          | 3.1 | 10          | 3.1 | 10          | 3.2 | 10          | 3.2 | 5           | 1.6 | 5           | 1.6 |
| Na <sub>2</sub> HPO <sub>4</sub> (sat'd sol'n) | 0.2         | —   | 0.2         | —   | 0.2         | —   | 0.2         | —   | 0.2         | —   | 0.2         | —   |
| Oxalic (sat'd sol'n)                           | 0.6         | —   | 0.6         | —   | 0.6         | —   | 0.6         | —   | 0.6         | —   | 0.6         | —   |
| Wetting agent                                  | 0.1         | —   | 0.1         | —   | 0.1         | —   | 0.1         | —   | 0.1         | —   | 0.1         | —   |
| H <sub>2</sub> O                               | 77.0        | —   | 77.0        | —   | 66.1        | —   | 66.1        | —   | 63.0        | —   | 63.0        | —   |
| Metal <sup>1</sup>                             | —           | —   | —           | —   | —           | —   | —           | —   | —           | —   | —           | —   |
| Temperature ° F                                | 70          | —   | 140         | —   | 70          | —   | 120         | —   | 100         | —   | 160         | —   |
| Milling rate (mils/min.)                       | 0.3—        | —   | 2.0+        | —   | 0.8+        | —   | 4.0+        | —   | 0.1+        | —   | 1.3—        | —   |
| R.M.S.                                         | 35-40       | —   | 47-53       | —   | 36-40       | —   | 50-55       | —   | 28-33       | —   | 41-47       | —   |

<sup>1</sup> A heat treated aluminum alloy such as 7075S-T6 having a weight of about 0.045 g./in.<sup>2</sup> mil.

Table VII

| Variable                                       | A           |     | B           |      | C           |      | D           |     | E           |      | F           |      | G           |      |
|------------------------------------------------|-------------|-----|-------------|------|-------------|------|-------------|-----|-------------|------|-------------|------|-------------|------|
|                                                | Wt. Percent | N   | Wt. Percent | N    | Wt. Percent | N    | Wt. Percent | N   | Wt. Percent | N    | Wt. Percent | N    | Wt. Percent | N    |
| HNO <sub>3</sub> (68-70%)                      | 20.4        | 2.5 | 20.3        | 2.5  | 20.0        | 2.4  | 19.2        | 2.4 | 18.8        | 2.3  | 18.8        | 2.3  | 18.8        | 2.3  |
| Acetic acid (glacial)                          | 2.3         | 0.4 | 2.3         | 0.4  | 2.3         | 0.4  | 2.2         | 0.4 | 2.1         | 0.4  | 2.1         | 0.4  | 2.1         | 0.4  |
| HCl (38%)                                      | 16.4        | 1.9 | 16.3        | 1.9  | 16.1        | 1.8  | 15.5        | 1.8 | 15.1        | 1.8  | 15.1        | 1.8  | 15.1        | 1.8  |
| HF (60%)                                       | 0           | —   | 0.9         | 0.25 | 2.5         | 0.76 | 6.1         | 2.0 | 8.0         | 2.65 | 8.0         | 2.65 | 8.0         | 2.65 |
| Citric acid (sat'd sol'n)                      | 0.9         | —   | 0.9         | —    | 0.8         | —    | 0.8         | —   | 0.8         | —    | 0.8         | —    | 0.8         | —    |
| Na <sub>2</sub> HPO <sub>4</sub> (sat'd sol'n) | 0.3         | —   | 0.3         | —    | 0.3         | —    | 0.3         | —   | 0.3         | —    | 0.3         | —    | 0.3         | —    |
| H <sub>2</sub> O                               | 59.6        | —   | 59.1        | —    | 58.2        | —    | 56.0        | —   | 54.8        | —    | 54.8        | —    | 54.8        | —    |
| Metal <sup>1</sup>                             | —           | —   | 140-137     | —    | 135-132     | —    | 132-134     | —   | 133-138     | —    | 133-136     | —    | 150-152.5   | —    |
| Temperature ° F                                | —           | —   | —           | —    | —           | —    | —           | —   | —           | —    | —           | —    | 121-122     | —    |
| Milling rate (mils/min.)                       | 0           | —   | 0.10        | —    | 1.7         | —    | 3.6         | —   | 3.8         | —    | 4.8         | —    | 1.8         | —    |
| R.M.S.                                         | —           | —   | —           | —    | 15          | —    | 15          | —   | 13          | —    | 18          | —    | 15          | —    |

<sup>1</sup> 6Al-4V-Ti, an alloy of titanium, aluminum and vanadium.

Fundamentally, the solutions of Table VII comprised nitric acid, acetic acid, hydrochloric acid, citric acid, disodium monohydrogen phosphate and water. The alloy upon which the chemical milling solutions were used was an alloy of titanium, more specifically, C-120AV, and generally referred to 6Al-4V-Ti. In solution A there was no hydrofluoric acid, and the milling temperature was about 140° F., and the milling rate was substantially zero. In solutions B, C, D and E the concentration of the hydrofluoric acid was increased to 0.25 normal, 0.76 normal, 2.0 normal, and 2.65 normal, respectively. The milling temperatures were in substantially the same range, viz., 132-138° F. As is appreciated for these solutions the milling rate increased with an increase in the concentration of the hydrofluoric acid. More particularly, for solution B the milling rate was 0.10 mil per minute, for C a milling rate of 1.7, for D a rate of 3.6, and for E a rate of 3.8. The surface roughness or R.M.S. values was approximately the same, in the range of 13-18. Again, this progressive rise in the milling rate with the progressive increase in the concentration of the hydrofluoric acid indicates that the hydrofluoric acid plays a very important role in the chemical milling. As a variation on solution E solutions F and G were

used for milling at different temperatures. Solutions E, F, and G were substantially the same. More particularly, solution F was used at a temperature of approximately 150° F. and solution G at a temperature of about 121° F. Contrasting the three solutions, E, F and G, it is seen that F milled more rapidly than E, 4.8 mils per minute to 3.8 mils per minute. Also, G milled more slowly than either E or F at the rate of 1.8 mils per minute. These figures are as expected as with the increase of temperature of F over E and G there was an increase in the milling rate for substantially the same fundamental solution. And, for a decrease of temperature, see G and E, there was a decrease in the milling rate. In summary, it can be said that an increase in the hydrofluoric acid concentration increases the milling rate and an increase in temperature increases the milling rate.

Turning now to another series of solutions comprising the components nitric acid, hydrochloric acid, acetic acid, hydrofluoric acid, citric acid, disodium monohydrogen phosphate and water, the results of chemical milling with this series of solutions are presented in the following Table VIII.

Table VIII

| Variable                                       | A                              |     | B                                        |     | C                                        |     | D                                        |     |
|------------------------------------------------|--------------------------------|-----|------------------------------------------|-----|------------------------------------------|-----|------------------------------------------|-----|
|                                                | Wt. Percent                    | N   | Wt. Percent                              | N   | Wt. Percent                              | N   | Wt. Percent                              | N   |
| HNO <sub>3</sub> (68-70%)                      | 23.8                           | 3.0 | 23.8                                     | 3.0 | 22.7                                     | 2.9 | 20.2                                     | 2.2 |
| HCl (38%)                                      | 5.2                            | 0.6 | 5.2                                      | 0.6 | 9.9                                      | 1.2 | 8.8                                      | 0.9 |
| Acetic acid (glacial)                          | 2.7                            | —   | 0.5                                      | —   | 2.3                                      | 0.5 | 2.3                                      | 0.4 |
| HF (60%)                                       | 9.5                            | 3.2 | 9.5                                      | 3.2 | 9.0                                      | 3.1 | 16.5                                     | 5.0 |
| Citric acid (sat'd sol'n)                      | 1.0                            | —   | 1.0                                      | —   | 1.0                                      | —   | 0.8                                      | —   |
| Na <sub>2</sub> HPO <sub>4</sub> (sat'd sol'n) | 0.3                            | —   | 0.3                                      | —   | 0.3                                      | —   | 0.3                                      | —   |
| H <sub>2</sub> O                               | 57.4                           | —   | 57.4                                     | —   | 54.5                                     | —   | 48.6                                     | —   |
| HBr (47%)                                      | —                              | —   | —                                        | —   | —                                        | —   | 2.4                                      | —   |
| Metal                                          | Ti, 17-7PH                     | —   | Ti, 17-7PH, 316                          | —   | Ti, 17-7PH, 316                          | —   | Ti, 17-7PH, 316                          | —   |
| Temperature ° F                                | 80                             | —   | 160                                      | —   | Room                                     | —   | Room                                     | —   |
| R.M.S.                                         | —                              | —   | 17-7PH, 70-85; 316, 40-60                | —   | Ti—Extremely fast; 17-7PH—Fast; 316—Fair | —   | Ti—Extremely fast; 17-7PH—Fast; 316—Fast | —   |
| Milling rate                                   | Ti—Very fast; 17-7PH—Fair-good | —   | Ti—Extremely fast; 17-7PH—Fast; 316—Fast | —   | Ti—Extremely fast; 17-7PH—Fast; 316—Fast | —   | Ti—Extremely fast; 17-7PH—Fast; 316—Fast | —   |

In Table VIII solutions A and B are comparable as they are substantially the same solutions with only the milling temperature differing, i.e., for A the milling temperature was 80° F. and for B the milling temperature was 160° F. The metals milled by these solutions were commercially pure titanium, 17-7PH steel and 316 steel. Solution A milled titanium very rapidly and milled 17-7PH steel rapidly although not as rapidly as the titanium. However, with an increase in the temperature from 80° to 160° F. solution B milled titanium extremely fast, milled 17-7PH steel fast, and reacted fairly fast on 316 steel although not as rapidly as on the 17-7PH. Studying the results of milling with A and B it is seen that with an increase in temperature the milling rate increased making it possible to more rapidly mill some metals at higher temperatures which would be practically impossible, economically speaking, to mill at lower temperatures. Solution C was a modification of solutions A and B in that the concentration of the hydrochloric acid was increased at the expense of the nitric acid, acetic acid, hydrofluoric acid present. The alloys milled by solution C were commercially pure titanium, 17-7PH steel and 316 steel. Again, solution C milled titanium extremely fast, and milled 17-7PH and 316 steel fast although not as rapidly as the titanium. Solution D comprised the same components as solutions A, B and C, but the concentration of the nitric acid was considerably lower being 2.2 normal, the hydrochloric acid was 0.9 normal, the acetic acid was substantially the same as for the other solutions, but the concentration of the hydrofluoric acid was increased to 5 normal. This solution was used for milling titanium, 17-7PH and 316 steels. With the titanium the solution milled extremely fast, with 17-7PH steel the solution was fast, and with 316 steel the solution was also fast. Referring again to Table VIII it is seen that the milling rate in this table is given in terms of a qualitative value and not in terms of a quantitative value. For this particular series of solutions the change in weight of the

the indicated metal. Then, to this solution there was added additional hydrofluoric acid to make solution B and additional metal milled. This was repeated for solutions C, D, E and F. As is readily realized there was a buildup of the reaction products between the metal and the reactant solution. So, in effect there were so many parts of the alloy in solution for each successive addition of the hydrofluoric acid to make a new solution. Referring again to solution A it is seen that at the start of this reaction there were zero parts of the metal in solution and at the end of the reaction there was 0.005 part per part of hydrofluoric acid present. The part of hydrofluoric acid present was based on the volume of the acid, the percent by weight (60%) and the specific gravity (1.19) of the acid. The weight of metal dissolved was known and therefore the ratio of part of metal to part of hydrofluoric acid was readily determined. With reference to the succeeding solution, for example, solution D, at the start of the milling reaction there were about 0.029 part of the alloy in the solution and at the end of the milling reaction there were about 0.033 part of alloy in the solution per part of the hydrofluoric acid. The temperature of milling solution was substantially at 130° F. or, more particularly,  $130 \pm 2$ ° F. The milling rates of these solutions were not identical but were in the same range. For example, solution A initially had a milling rate of 1.9 mils per minute and decreased to 1.0 mil per minute with buildup of the metal-solution product in the solution. Solution B had an initial rate of about 3.1 mils per minute and decreased to 2.4 mils per minute. Solution C started out at approximately 1.8 mils per minute and decreased to 1.2 mils per minute. Upon further addition of hydrofluoric acid, solution D initially had a milling rate of 2.3 mils per minute and decreased to 0.6 mil per minute. Similarly, solution E had an initial rate of 2.3 mils per minute and decreased to 1.2, and solution F had an initial rate of 2.1 mils per minute and decreased to 0.7 mil per minute.

Table IX

| Variable                                                 | A           |     | B           |     | C           |     | D           |     | E           |     | F           |     |
|----------------------------------------------------------|-------------|-----|-------------|-----|-------------|-----|-------------|-----|-------------|-----|-------------|-----|
|                                                          | Wt. Percent | N   | Wt. Percent | N   | Wt. Percent | N   | Wt. Percent | N   | Wt. Percent | N   | Wt. Percent | N   |
| HNO <sub>3</sub> (68-70%)                                | 19.2        | 2.4 | 18.4        | 2.3 | 18.2        | 2.3 | 17.9        | 2.2 | 17.6        | 2.2 | 17.4        | 2.2 |
| Acetic acid (glacial)                                    | 2.2         | 0.4 | 2.1         | 0.4 | 2.0         | 0.4 | 2.0         | 0.4 | 2.0         | 0.4 | 2.0         | 0.4 |
| HCl (35%)                                                | 15.5        | 1.8 | 14.8        | 1.7 | 14.6        | 1.7 | 14.4        | 1.7 | 14.3        | 1.6 | 14.0        | 1.6 |
| HF (60%)                                                 | 6.1         | 2.0 | 9.8         | 3.3 | 11.2        | 3.7 | 12.5        | 4.2 | 13.8        | 4.7 | 15.1        | 5.1 |
| Citric acid (sat'd sol'n.)                               | 0.8         | —   | 0.8         | —   | 0.8         | —   | 0.8         | —   | 0.7         | —   | 0.7         | —   |
| Na <sub>2</sub> HPO <sub>4</sub> (sat'd sol'n.)          | 0.3         | —   | 0.3         | —   | 0.3         | —   | 0.3         | —   | 0.3         | —   | 0.2         | —   |
| H <sub>2</sub> O                                         | 56.0        | —   | 53.8        | —   | 53.0        | —   | 52.2        | —   | 51.4        | —   | 50.7        | —   |
| Metal                                                    | 6A1-4V-T1   | —   | 6A1-4V-T1   | —   | 6A1-4V-T1   | —   | 6A1-4V-T1   | —   | 6A1-4V-T1   | —   | 6A1-4V-T1   | —   |
| Temperature ° F.                                         | 130±2       | —   | 130±2       | —   | 130±2       | —   | 130±2       | —   | 130±2       | —   | 130±2       | —   |
| Milling rate mils/min.                                   | 1.0-1.9     | —   | 2.4-3.1     | —   | 1.2-1.8     | —   | 0.6-2.3     | —   | 1.2-2.3     | —   | 0.7-2.1     | —   |
| Start of reaction—part metal in sol'n per part of sol'n. | 0           | —   | 0.005       | —   | 0.017       | —   | 0.029       | —   | 0.034       | —   | 0.039       | —   |
| End of reaction—part metal in sol'n per part of sol'n.   | 0.005       | —   | 0.009       | —   | 0.028       | —   | 0.033       | —   | 0.039       | —   | 0.047       | —   |

metals milled was not determined. Therefore, a qualitative determination of the milling rate was used. From this table it is seen that an increase in temperature increases the milling rate, that an increase in the concentration of the hydrochloric acid and the hydrofluoric acid present also increases the milling rate.

Another milling solution was prepared, see following Table IX, comprising nitric acid, acetic acid, hydrochloric acid, hydrofluoric acid, citric acid, disodium monohydrogen phosphate, and water. The fundamental solution was varied by increasing the concentration of the hydrofluoric acid present so that the range of hydrofluoric acid covered from 2.0 normal to about 5.1 normal. More particularly, in this series of milling solutions a titanium alloy, said alloy being 6Al-4V-Ti, was milled by these solutions. The weakest solution with respect to the hydrofluoric acid present, see solution A, was used to mill

Additional information was found for solutions A and F in that the milling rate for the various parts of metal in the solution per part of the hydrofluoric acid originally present was determined. This information is recorded in column form in Table X. Referring to the table it is seen that for solution A with no metal dissolved in the solution the initial milling rate was approximately 1.63 mils per minute. Upon the dissolving of the metal in the solution the milling rate momentarily increased to 1.88 and then leveled off at approximately 1.75 mils per minute until the concentration of the products in the solution reached approximately 0.05 part of metal per part of hydrofluoric acid. After this time, and also upon the increase in concentration of the metal, in the hydrofluoric acid, the reaction rate decreased to 1.67 mils per minute or approximately 1.7, then decreased to 1.5, 1.25, 75 and finally to about 1.0 mil per minute. Turning now to

solution F it is seen that with a concentration of the metal in the solution of approximately 0.26 part metal to each part of hydrofluoric acid the milling rate was about 2.1 mils per minute. With the buildup of the concentration of the metal to about 0.3 the milling rate was about 1.1 and with a further buildup of the metal the milling rate decreased to about 0.75. A plot of these milling rates is in Figure 8. From this graph it is seen that for solution A there is a rather long and uniform milling rate based upon the buildup of the metal in the solution. However, for solution F it is noticed that the reaction rate decreased rapidly. From this information it is hypothesized that the concentration of the weak acid in the solution such as the combination of the acetic and the citric acid determines to a large degree the uniformity of the milling rate of the solution. For example, with solution A the ratio of the volume of the glacial acetic acid and the saturated citric solutions to the total volume of the solution was 0.032 part per part, and for solution F this same ratio was 0.022 part per part. From this it is possible to state that the presence of a weak acid such as citric acid, acetic acid, oxalic acid, and boric acid having a primary ionization constant in the range of  $10^{-4}$  to  $10^{-6}$  moderate the reaction so that it assumes a longer uniform rate of reaction. Below a certain volume concentration of these indicated weak acids the reaction starts out at a high rate and rapidly decreases to a low rate. Above a certain minimum concentration of these acids the reaction rate of the solution was relatively uniform and instead of precipitously decreasing the reaction rate decreased slowly. In fact, the reaction rate may be considered to be on a plateau for a long period. Naturally it is readily realized that an advantage of this type of reaction is the closer controlling of the same. With the uniform reaction it is possible to control the reaction and the eating away of the metal so that a more uniform product can be realized. As contrasted with this a reaction which starts out at a high rate and rapidly decreases to a low rate is more difficult to control so as to predict the time period in which the metal should be immersed in the solution in order to achieve the proper amount of metal removal.

Table X  
SOLUTION A  
[Parts by weight HF = 6.1%]

| Milling Rate mils/min. | Parts at Start | Parts Metal/Parts HF |
|------------------------|----------------|----------------------|
| 1.63                   | 0              | 0                    |
| 1.88                   | 7.5            | 0.014                |
| 1.75                   | 15.8           | 0.030                |
| 1.75                   | 24.2           | 0.045                |
| 1.75                   | 33.4           | 0.062                |
| 1.67                   | 47.1           | 0.088                |
| 1.50                   | 58.3           | 0.110                |
| 1.25                   | 62.1           | 0.116                |
| 1.00                   | 71.9           | 0.134                |

NOTE.—Ratio of acetic plus citric acid solution to total volume of solution equals 0.032.

SOLUTION F  
[Parts by weight HF = 15.1%]

| Milling Rate mils/min. | Parts at Start | Parts Metal/Parts HF |
|------------------------|----------------|----------------------|
| 2.125                  | 630.5          | 0.258                |
| 1.13                   | 720.1          | 0.296                |
| 0.88                   | 736.1          | 0.302                |
| 0.75                   | 750.7          | 0.308                |

NOTE.—Ratio of acetic plus citric acid solution to total volume of solution equals 0.022.

20  
Table XI

| Variable                                        | A                                         |                                                | B                                                                                     |                                                                                       |
|-------------------------------------------------|-------------------------------------------|------------------------------------------------|---------------------------------------------------------------------------------------|---------------------------------------------------------------------------------------|
|                                                 | Wt. Percent                               | N                                              | Wt. Percent                                                                           | N                                                                                     |
| HNO <sub>3</sub> (68-70%)                       | 19.2                                      | 2.4                                            | 19.2                                                                                  | 2.4                                                                                   |
| Acetic acid (glacial)                           | 2.2                                       | 0.4                                            | 2.2                                                                                   | 0.4                                                                                   |
| HCl (38%)                                       | 8.4                                       | 1.0                                            | 8.4                                                                                   | 1.0                                                                                   |
| HF (60%)                                        | 15.6                                      | 5.3                                            | 15.6                                                                                  | 5.3                                                                                   |
| HBr (47%)                                       | 4.7                                       | 0.3                                            | 4.7                                                                                   | 0.3                                                                                   |
| Citric acid (sat'd sol'n.)                      | 0.8                                       | —                                              | 0.8                                                                                   | —                                                                                     |
| Na <sub>2</sub> HPO <sub>4</sub> (sat'd sol'n.) | 0.2                                       | —                                              | 0.2                                                                                   | —                                                                                     |
| H <sub>2</sub> O                                | 48.8                                      | —                                              | 48.8                                                                                  | —                                                                                     |
| Metal                                           | Ti, 17-7PH; 6Al-4V-Ti                     | 6Al-4V-Ti; Ti, 17-7PH, AM350                   | Ti, 17-7PH; 6Al-4V-Ti                                                                 | Ti, 17-7PH, AM350                                                                     |
| Temperature °F                                  | 80                                        | —                                              | 160                                                                                   | —                                                                                     |
| Milling rate                                    | Ti and 6Al-4V-Ti—Very rapid; 17-7PH—Rapid | AM-350, good; Ti, 17-7PH, 6Al-4V-Ti—Very rapid | Ti, 8-11—As rolled; 50-60; 6Al-4V-Ti, 4-6—As rolled; 100-120; 17-7PH, 45—As rolled 50 | Ti, 8-11—As rolled; 50-60; 6Al-4V-Ti, 4-6—As rolled; 100-120; 17-7PH, 45—As rolled 50 |
| RMS                                             | —                                         | —                                              | —                                                                                     | —                                                                                     |

Table XI summarizes in a qualitative manner the reaction rate of a typical solution on various metals and also the R.M.S. value of these metals both before and after milling. The solution comprised nitric acid, acetic acid, hydrochloric acid, hydrofluoric acid, hydrobromic acid, citric acid, disodium monohydrogen phosphate and water. The presence of the hydrofluoric acid was in the range of approximately 5.3 normal, the nitric acid about 2.4 normal, and the hydrochloric acid about 1.0 normal. At 80° F. the solution, see A, reacted very rapidly with pure titanium and an alloy of 6Al-4V-Ti, and reacted rapidly on 17-7PH steel. At 160° F. the same solution reacted at a good rate with AM350 steel, and reacted very rapidly with pure titanium, 17-7PH steel and 6Al-4V-Ti. In regard to the R.M.S. values for titanium the as rolled value was in the range of 50 to 60 while the milled metal value was in the range of 8 to 11. For 6Al-4V-Ti the as rolled values were in the range of 100 to 120 while the milled metal value was in the range of 4 to 6. And, with 17-7PH the as rolled value was about 50 while the corroded value was 45. This reaction solution produced a surface on metal which was extremely smooth, for example, see titanium and the alloy of titanium having values in the range of 8-11 and 4-6 respectively. The 17-7PH milled metal was also somewhat smoother than the as rolled metal.

In Table XII there is presented another fundamental milling solution with variations thereof. Fundamentally, this solution comprised nitric acid, hydrochloric acid, acetic acid, hydrofluoric acid, and water. The nitric acid was about 4.7 normal and the hydrofluoric acid about 1.4 normal. At approximately room temperature solution A reacted very rapidly with 17-7PH. To this solution there was added citric acid and disodium monohydrogen phosphate to form solution B. Solution B was used for milling 17-7PH steel and it was found that fast milling was achieved with this solution. However, it was observed that B did not mill as rapidly as A. This indicates that the addition of the citric acid and disodium monohydrogen phosphate moderated the milling action. This moderating action comprised slowing down the reaction rate so as to more closely regulate the reaction. To a solution such as solution B there was added additional citric acid and a complex salt of ammonium fluoride and hydrogen fluoride. As contrasted with solutions A and B solution C was used to mill both 17-7PH and 6Al-4V-Ti. With each of these metals solution C did a rapid milling job.

Table XII

| Variable                                        | A                             |     | B                       |                                       | C           |     |
|-------------------------------------------------|-------------------------------|-----|-------------------------|---------------------------------------|-------------|-----|
|                                                 | Wt. Percent                   | N   | Wt. Percent             | N                                     | Wt. Percent | N   |
| HNO <sub>3</sub> (68-70%)                       | 36.7                          | 4.7 | 36.2                    | 4.7                                   | 35.6        | 4.7 |
| HCl (38%)                                       | 9.0                           | 1.1 | 9.0                     | 1.1                                   | 8.8         | 1.1 |
| Acetic acid (glacial)                           | 2.8                           | 0.5 | 2.7                     | 0.5                                   | 2.6         | 0.5 |
| HF (60%)                                        | 4.1                           | 1.4 | 4.1                     | 1.4                                   | 4.0         | 1.5 |
| H <sub>2</sub> O                                | 47.4                          |     | 46.9                    |                                       | 45.9        |     |
| Citric acid (sat'd sol'n.)                      |                               |     | 1.0                     |                                       | 1.8         |     |
| Na <sub>2</sub> HPO <sub>4</sub> (sat'd sol'n.) |                               |     | 0.3                     |                                       | 0.3         |     |
| NH <sub>4</sub> F.HF                            |                               |     |                         |                                       | 0.8         |     |
| Temperature ° F                                 | Room                          |     | Slow milling of 17-7PH. |                                       | Room        |     |
| Metal                                           | Very rapid milling of 17-7PH. |     |                         | Fast milling of 17-7PH and 6Al-4V-Ti. |             |     |

the milling rate 0.5 mil per minute, and the R.M.S. value about 12. Again, a comparison of B with B, or approximately same milling temperatures and with an increase in nitric acid concentration and a decrease in hydrofluoric concentration there was apparently a synergistic effect tending to lower the milling rate of the solution. And, in solution E the nitric acid was about 3.9 normal, the hydrochloric about 0.6 normal and the hydrofluoric about 5.2 normal. The milling temperature was 90° F., the milling rate 2.0 mils per minute and the R.M.S., 9. A comparison of E with C, whereby the two were at substantially the same milling temperature, shows that even though there is an increase in the nitric acid concentration that if there is a sufficient increase in the hydrofluoric acid concentration there will then be a rapid milling rate. An overall view of these compositions, A, B, C, D, and E indicates that with the raising of the concen-

Table XIII

| Variable                                        | A           |      | B           |      | C           |      | D           |      | E           |      |
|-------------------------------------------------|-------------|------|-------------|------|-------------|------|-------------|------|-------------|------|
|                                                 | Wt. Percent | N    | Wt. Percent | N    | Wt. Percent | N    | Wt. Percent | N    | Wt. Percent | N    |
| HNO <sub>3</sub> (68-70%)                       | 1           | 0.1  | 1           | 0.1  | 8           | 0.9  | 10          | 1.2  | 30          | 3.9  |
| HCl (38%)                                       | 10          | 1.1  | 10          | 1.1  | 5           | 0.5  | 10          | 1.1  | 5           | 0.6  |
| Acetic acid (glacial)                           | 3           | 0.5  | 3           | 0.5  | 3           | 0.5  | 3           | 0.5  | 5           | 1.0  |
| HF (60%)                                        | 10          | 3.1  | 10          | 3.1  | 8           | 2.5  | 2           | 0.6  | 15          | 5.2  |
| NH <sub>4</sub> F.HF                            |             |      |             |      |             |      | 2           | .4   |             |      |
| Na <sub>2</sub> HPO <sub>4</sub> (sat'd sol'n.) | 0.4         |      | 0.4         |      | 0.4         |      | 0.4         |      | 0.4         |      |
| Boric acid (sat'd sol'n.)                       | 1.2         |      | 1.2         |      | 1.2         |      |             |      |             |      |
| Citric acid (sat'd sol'n.)                      |             |      |             |      |             |      | 1.2         |      | 1.2         |      |
| Wetting agent                                   |             | 0.1  |             | 0.1  |             | 0.1  |             | 0.1  |             | 0.1  |
| H <sub>2</sub> O                                |             | 74.2 |             | 74.2 |             | 74.2 |             | 71.1 |             | 43.2 |
| Temperature ° F                                 | 80.         |      | 120.        |      | 90.         |      | 135.        |      | 90.         |      |
| Milling rate (mils/min.)                        | 0.5         |      | 2.5         |      | 0.3         |      | 0.5         |      | 2.0         |      |
| RMS                                             | 15.         |      | 10.         |      | 16.         |      | 12.         |      | 9.          |      |
| Metal                                           | 6Al-4V-Ti   |      | 6Al-4V-Ti   |      | 6Al-4V-Ti   |      | 6Al-4V-Ti   |      | 6Al-4V-Ti   |      |

Another set of milling solutions for the milling of titanium was prepared (see Table XIII). These solutions comprised nitric acid, hydrochloric acid, acetic acid, hydrofluoric acid, ammonium bifluoride, disodium monohydrogen phosphate, boric acid, citric acid, a wetting agent such as the sodium salt of the sulfonic acid of dodecyl benzene, and water. The boric acid solution was prepared by heating water to the boiling temperature, adding an excess of boric acid, cooling and decanting the saturated boric acid solution. The metal milled by the solutions was a titanium alloy such as 6Al-4V-Ti. Solutions A and B were the same except that solution A was used for milling at 80° F. and B at 120° F. In these solutions the concentration of nitric acid was 0.1 normal, the hydrochloric 1.1 normal and the hydrofluoric about 3.1 normal. The milling rate for solution A was 0.5 mil per minute and for solution B about 2.5 mils per minute and the R.M.S. value for A was 15 and for B, 10. It is seen that a relatively modest increase in temperature from A to B in a solution comprising a relatively high concentration of hydrofluoric acid produced a large increase in the milling rate. Attention is called to the fact that nitric acid concentration was rather low, 0.1 normal, in solutions A and B. In solution C the nitric acid concentration was raised to about 0.9 normal, hydrochloric lowered to 0.5 normal and hydrofluoric acid decreased to 2.5 normal. The milling temperature was 90° F. and the milling rate 0.3 mils per minute, the R.M.S. value 16. A comparison of C with A shows a decrease in the milling rate. It can be surmised that the corresponding increase in the concentration of the nitric acid and the corresponding decrease in the concentration of the hydrofluoric acid produced a synergistic effect so as to lower the milling rate of solution C with respect to solution A even though the temperatures were approximately the same. In solution D the nitric acid concentration was about 1.2 normal, the hydrochloric acid 1.1 normal and the hydrofluoric about 0.6 normal. The milling temperature was 135° F.,

40 tration of the nitric acid and the lowering of the hydrofluoric acid concentration there is a decrease in the milling rate. However, if both the nitric acid concentration and the hydrofluoric acid concentration be raised, particularly the latter, there is an increase in the milling rate.

Having described our discovery and illustrated the same with reference to various compositions of matter for the use of chemical milling solution, reference is hereby made to the practical application of these solutions. Referring to the drawings, and especially Figure 1, it is seen that there is illustrated a structural panel 10 having two chemically milled recesses 11 therein. In Figure 2, a vertical cross-sectional view of Figure 1, it is seen that this structural panel is curved and that these two recesses are separated from each other by a rib 12. In the manufacture of this type of structural panel the material to be saved is covered by an adhering and strippable protective film or coating, there are numerous such coatings or films examples being neoprene, vinyl etch-proof film, and others. More particularly, for shallow milling there may be used various acid resistant paints. To pictorially illustrate the making of this structural panel reference is made to Figures 3 and 4. In Figure 3 there is illustrated a neoprene mask 13 having two recesses 14 therein. This neoprene film 13 is placed on the concave side of the structural panel 10 and on the edges and the convex side are attached other protective neoprene films. A cross-sectional view of the structural panel before chemical milling takes place is shown in Figure 4 whereby the panel is covered by the neoprene having the two cutouts 14 illustrated therein. This structural panel is now ready to be chemically milled and is dipped or submerged in the milling solution for a predetermined time. With the 50 passing of the time the milling solution eats away or corrodes away the metal so as to form the two recesses 11. It is to be noted that that portion of the metal covered by the protective neoprene film is not attacked and only that portion of the metal not covered by the protective film is corroded away. After the passage of a predetermined

mined period of time and the recesses are of a sufficient depth and size the structural panel is removed from the milling solution. The adherent solution is washed away and the neoprene protective film stripped off the panel to produce that shown in Figure 1. Other teachings for the masking of metal may be found in United States Patents Numbers 2,739,047 to Sanz and 2,684,291 to Wilson et al.

In Figure 5 there is illustrated the action of the milling solution on the metal at the junction of the protective film and the metal. It is seen that milling solution 16 eats away metal 17 so as to undercut protective film 18. One of the particular advantages of the use of a wetting agent is to induce better contact between the milling solution and the metal. With a better contact or a lowering of the effective surface tension there is less possibility of gases collecting on the surface or near masked edges underneath the protective film. For this function there are a number of suitable wetting agents such as pine oil. One of the common wetting agents is an alkyl aryl sulfonate. Specific sulfonates which are useful are the sodium salts of dodecyl benzene sulfonic acid and pentadecyl benzene sulfonic acid.

Another instance where our solution is of value is in the chemical milling of components for aircraft. In Figure 6 is illustrated a curved structural plate having a thickness of 0.61 inch. This plate was transformed into a structural member, for use in a fuel tank, having a thickness of 0.100 inch, outside dimensions of eight inches square, a circular boss in the center of three inches in diameter and of the original thickness of 0.610 inch. The finished product was prepared from the original structural plate by masking the central portion on each side so as to form the boss upon the corrosion of the rest of the metal. Normally, such a metal would be formed by fabrication using welding techniques. The welding process causes grain growth which in turn causes a weakening of the metal. With our method there is no grain growth.

The control for determining the degree of chemical milling may be carried out in a number of different manners. One of these is to introduce a material of a predetermined thickness into the chemical milling solution along with the member to be chemically milled and to periodically weigh or measure this member. When this member has decreased a certain amount in weight or thickness it is possible to decide whether the structural member undergoing chemical milling has been corroded away sufficiently.

Returning now to the tables and the examples presented therein it is noticed that the smoothness or R.M.S. values are in the range of approximately 20 to 45 R.M.S. This is of a special importance as this value represents a surface that is relatively smooth. In fact, the milled metal is often smoother than the metal when machined milled. In machine milling the average smoothness value is approximately 125 R.M.S. Of course, this value of 125 R.M.S. is subject to variation as with soft alloys it is possible to machine mill the metal somewhat smoother than 125 R.M.S., but with heat treated, work hardened, and tempered alloys which may have a tough surface skin it is difficult to achieve a smoothness value of 125 R.M.S. on machine milling. However, with this chemical milling process it is possible to achieve a smoothness value which approaches that used for reflective surfaces, and it is possible to achieve this smoothness on all types of alloys be they hard, heat treated, work hardened, or tempered.

The smoothness values were determined by a profilometer. The profilometer used possessed a diamond needle which rode on the surface of a metal and measured the profile of the surface in millionths of an inch in amplitude. These measurements are expressed in R.M.S. or root mean square values. Such an instrument is commercially obtainable from Physicists Research Co., Ann Arbor, Michigan.

In this chemical milling process it is noticed that there is little if any smut. Smut is defined as that material which clings to the metal itself. Smut is usually an oxide of the alloy or chemical compounds of the alloy or unreacted finely divided alloying materials and is attracted to the bulk metal by electrochemical and electrostatic forces.

With our process and chemical milling solution it is possible to achieve tolerances in some usages which have not been attainable in commercial practice before. These tolerances are in the range of approximately plus or minus 0.0005 inch, making it possible to achieve a high quality and/or a precision product. Also, in our process it has been observed that there is no intergranular corrosion due to the chemical action of the solutions. This success in not having intergranular corrosion makes it possible to achieve higher strength components for less weight of the component as compared with the presently machined milled and welded components.

Our process is also adaptable for a continuous method or a batch method. In the continuous process it is possible to contact the structural item to be made with a milling solution and to continuously recirculate the milling solution so as to maintain uniformity of solution in contact with all reacting surfaces. Chemical processing equipment, i.e., tanks, pipe fittings, valves, and pumps lined with a suitable resistant material such as polyethylene, polyvinylchloride, and polyvinylesters, capable of withstanding the chemical action of these solutions are available. Also, filter screens and heat exchange equipment to withstand the chemical action of these solutions are available. Therefore, it is possible to maintain close solution control necessary for continuous operation.

Examples of other ways and means for chemically milling metals are herewith presented. A metal may be removed by spraying the solution onto it so as to have a fine stream of the reactant solution contact the metal. By this technique deep grooving can be realized by rotating a part. In another manner a pipe may be made lighter-in-weight by running the solution through it so as to decrease the wall thickness. As is realized the interior wall of the pipe is eaten away and the inside diameter thereby enlarged.

From the above description of our discovery it is seen that the same is applicable to the chemical milling of metal and alloys. From our discovery it is possible to save considerable weight in the manufacture of metal products; to produce the parts in batches or continuously; the capital investment for production of the components may be as low as approximately five to ten percent of the capital investment for equivalent machine milling. Also, it is possible to produce highly complex shapes and configurations with chemical milling which are not possible with machine milling, to use non-symmetrical patterns with chemical milling which are difficult to use with machine milling, to produce integrally stiffened structures whereby one unit serves as the structure instead of an integrally fabricated structure depending upon welds, which are weaker than the metal itself, to produce the structure, and to make tapered structural materials which are difficult to make with machine milling. Furthermore, from an engineering design standpoint it is seen that it is possible to etch after forming the structure. In many operations it is economically feasible to obtain closer tolerances, to have a number of various depths of cut, and to mill all surfaces of the part simultaneously. In this regard, it is possible to chemically mill with equal ease all types of aluminum and titanium and their alloys. From a labor standpoint and skilled artisan viewpoint it is not necessary in chemical milling to use as highly skilled operators as in machine milling.

Having described our discovery what we claim and wish to protect is as follows:

1. A composition of matter adapted for chemically milling metals which consists essentially of an aqueous

acidic medium containing a nitrate in the concentration range of about 0.1-4.7 molar, a chloride in the concentration range of about 0.1-2.2 molar, a fluoride in the concentration range of about 0.25-5.3 molar, and an acetate in a concentration of at least 0.22 normal, the aqueous medium as a whole having an available hydrogen ion concentration in the concentration range of about 2.8-10.7 molar.

2. A process for chemically milling a metal selected from the group consisting of aluminum, titanium, steel and alloys of these metals, said process comprising subjecting these metals to the action of a composition of matter which consists essentially of an aqueous acidic medium containing a nitrate in the concentration range of about 0.1-4.7 molar, a chloride in the concentration of about 0.1-2.2 molar, a fluoride in the concentration range of about 0.25-5.3 molar, and an acetate in a concentration of at least 0.22 normal, the aqueous medium as a whole having an available hydrogen ion concentration in the concentration range of about 2.8-10.7 molar.

3. A composition of matter adapted for chemically milling metals comprising an aqueous acidic medium containing a nitrate, a chloride, a fluoride, and minor amounts of a phosphate and a weak acid having an ionization constant in the range of  $10^{-4}$  to  $10^{-6}$ , the concentration of the nitrate and the chloride each being at least about 0.1 molar, the concentration of the fluoride being at least about 0.2 molar, and the aqueous medium as a whole having a available hydrogen ion concentration at least equivalent to about 2.8 molar.

4. A composition of matter adapted for chemically milling metals comprising an aqueous acidic medium containing a nitrate in the concentration range of about 0.1-4.7 molar, a chloride in the concentration range of about 0.1-2.2 molar, a fluoride in the concentration range of about 0.2-5.3 molar, and minor amounts of a phosphate and an acetate in a concentration of at least about 0.22 normal, the aqueous medium as a whole having an available hydrogen ion concentration in the range of about 2.8-10.7 molar.

5. A process for chemically milling a metal selected from the group consisting of aluminum, titanium, steel and alloys of these metals, said process comprising subjecting these metals to the action of an aqueous acidic medium containing nitric acid, hydrochloric acid, hydrofluoric acid, the concentration of nitric acid and hydrochloric acid each being at least about 0.1 molar, the con-

centration of hydrofluoric acid being at least about 0.2 molar, and minor amounts of a phosphate and a weak acid having an ionization constant in the range of  $10^{-4}$  to  $10^{-6}$ , the aqueous medium as a whole having an available hydrogen ion concentration in the concentration range of about 2.8-10.7 molar, and maintaining the temperature of treatment at between about room temperature and 210° F.

6. A composition of matter adapted for chemically

10 milling a metal selected from the group consisting of aluminum, titanium, steel and alloys of these metals, and which consists essentially of an aqueous acidic medium containing a nitrate, a chloride, a fluoride and an acetate, the concentration of the nitrate and chloride each being

15 at least about 0.1 normal, the concentration of the fluoride being at least about 0.25 normal, the concentration of the acetate being at least about 0.22 normal, the available hydrogen ion concentration being, however, at least 2.8 normal.

20 7. The composition of claim 6 wherein minor amounts of phosphate and citrate are present in said composition.

8. A process for chemically milling a metal selected from the group consisting of aluminum, titanium, steel and alloys of these metals, said process comprising sub-

25 jecting the metal to the action of a composition consisting essentially of an aqueous acidic medium containing a nitrate, a chloride, a fluoride and an acetate, the concentration of the nitrate and chloride each being at least about 0.1 normal, the concentration of the fluoride being

30 at least about 0.25 normal, the concentration of the acetate being at least about 0.22 normal, the available hydrogen ion concentration being, however, at least 2.8 normal.

9. The process of claim 8 wherein the temperature of

35 treatment is maintained at between about room tem-

perature and 210° F.

#### References Cited in the file of this patent

#### UNITED STATES PATENTS

|    |           |             |               |
|----|-----------|-------------|---------------|
| 40 | 2,337,062 | Page        | Dec. 21, 1943 |
|    | 2,374,070 | Barensfield | Apr. 17, 1945 |
|    | 2,446,060 | Pray et al. | July 27, 1948 |
|    | 2,662,814 | Swihart     | Dec. 15, 1953 |
| 45 | 2,739,047 | Sanz        | Mar. 20, 1956 |
|    | 2,828,192 | Langsfield  | Mar. 25, 1958 |
|    | 2,890,944 | Hays        | June 16, 1959 |